

## UNITED STATES PATENT OFFICE

WINFRID HENTRICH AND MAX HARDTMANN, OF WIESDORF-ON-THE-RHINE, JOSEF HILGER, OF COLOGNE-MULHEIM, AND RUDOLF KNOCHE, OF LEVERKUSEN-ON-THE-RHINE, GERMANY, ASSIGNORS TO GENERAL ANILINE WORKS, INC., OF NEW YORK, N. Y., A CORPORATION OF DELAWARE

## DYEING OF VISCOSE

No Drawing. Application filed February 26, 1929, Serial No. 342,956, and in Germany February 27, 1928.

The present invention relates to a process of producing even dyeings on viscose fabrics containing or composed of viscose of irregular physical or chemical quality and to the dyed fabrics obtainable thereby.

In dyeing viscose fabrics by means of the dyestuffs hitherto in use, streaky uneven dyeings are frequently obtained. This disadvantage is due to the irregular physical or chemical quality of the commercial viscose used, which displays a very variable affinity towards one and the same dyestuff.

In accordance with the present invention, the disadvantages encountered in the dyeing of viscose fabrics of irregular quality with the substantive dyestuffs hitherto employed, can be avoided by effecting the dyeing by means of dyestuffs containing, in complex combination, heavy metals, such as copper, nickel, cobalt, chromium, cadmium, zinc, vanadium and iron.

The azo dyestuffs which are capable of forming heavy metal complex compounds are distinguished by having a salicyclic group in the molecule or by having in ortho position to an azo group a hydroxy-, a carboxylic acid-, an alkoxy-, an aralkoxy- or an aldehyde-group.

The heavy metal complex compounds are generally obtainable by treating for some hours the aqueous solution of the dyestuff with an aqueous solution of a salt of the respective heavy metal. For example, dyestuffs, containing copper or iron, are obtainable by heating an aqueous solution of the dyestuff with copper sulfate or ferrous sulfate for several hours, or according to the process described in the U. S. P. 1,690,782, issued November 6, 1928 by reacting upon the aqueous solution of the dyestuff with a copper-amine compound.

Complex nickel, cobalt, cadmium or zinc amine azo compounds are obtainable, for example, by the use of nickelous amine salts, such a nickelous tetramine sulfate, of cobalt amine salts, such as carbonato tetramine cobalt chloride, or of cadmium- or zinc-amine salts, instead of the copper amine complex salts used in the process of U. S. P. 1,690,782.

Dyestuffs, containing chromium, are ob-

tainable by boiling the aqueous solution of the dyestuff for several hours with a water soluble chromium salt, such as chromium formate, and chromium fluoride; complex vanadium compounds are obtainable by boiling the dyestuff with a water soluble vanadic acid salt, for example, the ammonium salt of the meta vanadic acid.

The dyeing is carried out in the usual manner as is outlined in the examples, by dissolving the dyestuffs in hot water and adding to the dye-bath Glauber's salt and monopol soap (alkali metal salt of sulfonated castor oil), if desired with the addition of a wetting agent, f. i. an alkyl-naphthalene-sulfonic acid, such as iso butyl-naphthalene-disulfonic acid. The viscose is introduced into the bath at about 30° C., then the bath is slowly heated to about 80° C., at which temperature the viscose is dyed for about 3/4 hour to 1 hour. Then the viscose is washed and dried.

The dyeings thus produced on viscose and in particular on knitted artificial silk by means of the azo dyestuffs containing a heavy metal in complex combination possess a good fastness to light and are distinguished by an excellent evenness.

The following examples will illustrate our invention, without limiting it thereto:

*Example 1.*—2 g. of the dyestuff containing copper in complex combination, obtainable according to the process of the U. S. P. 1,690,782 from amino benzene-2-carboxylic acid, 2-phenylamino-5-hydroxy-naphthalene-7-sulfonic acid and tetramine-cupric sulfate and corresponding to the following probable formula:



are dissolved in 3 liters of hot water. 100 grams of knitted viscose are dyed for 1 hour at 80° C. in the presence of 20% of sodium sulfate and 2% of soap (calculated on the weight of the viscose). There is thus produced a beautiful and powerful ruby dyeing of excellent evenness, both in light and dark 100

dyeings, and of remarkable fastness to light.

The dyestuff obtainable from amino benzene-2-carboxylic acid and 2-benzoyl amino-5-hydroxynaphthalene-7-sulfonic acid and coppered in substance dyes, according to the same process, yellowish red shades; the copper amine complex compound of the dyestuff obtainable from 2 molecules of amino benzene-2-carboxylic acid, the urea of 2-amino-5-hydroxynaphthalene-7-sulfonic acid and tetramine-cupric sulfate dyes orange red shades; the copper amine complex compound of the dyestuff obtainable from two molecules of 4-chloro-1-amino benzene-2-carboxylic acid, 5,5'-dihydroxy-2,2'-dinaphthyl amine-7,7'-disulfonic acid and tetramine cupric sulfate dyes bluish violet shades. All these dyestuffs yield dyeings, which are very fast to light and distinguished by remarkable evenness.

A violet shade of the same properties is produced by dyeing knitted viscose artificial silk in the manner described with a dyestuff containing copper in complex combination and obtained from 5-nitro-2-amino-1-methoxy benzene-4-sulfonic acid and 2(4'-methoxy benzoyl)-amino-5-hydroxynaphthalene-7-sulfonic acid.

A remarkable even scarlet red dyeing is produced by the use of a dyestuff containing copper in complex combination and obtained from 2-amino-1-phenol glycerine ether and 2-(4'-methyl-benzoyl)-amino-5-hydroxy naphthalene-7-sulfonic acid.

Instead of the azo dyestuffs containing a carboxylic group in the ortho position to the azo group there can also be used quite generally such dyestuffs as contain the carbonyl- or hydroxy group in the ortho position to at least one azo group; the above mentioned dyestuffs containing a methoxy group in the ortho position to an azo group can likewise be replaced by dyestuffs, containing in the ortho position to an azo group other alkyl hydroxy-, aralkyl hydroxy- or aryl hydroxy groups, which may also be substituted, if desired.

*Example 2.*—By means of the dyestuff containing nickel in complex combination and obtained from 6-amino-1-hydroxy benzene-2-carboxylic acid, 1-amino naphthalene, 1-hydroxy naphthalene-5-sulfonic acid and nickel tetramine sulfate which dyestuff probably corresponds to the following formula:



applied to knitted viscose artificial silk in the manner described in Example 1 with the addition of 1% of isobutyl naphthalene sulfonic acid (calculated on the weight of the

material) a completely even bluish black dyeing is produced, possessing excellent fastness to light. The same dyestuff containing cobalt in complex combination yields a greenish black shade of similar properties.

Instead of the dyestuffs here specifically described, other dyestuffs containing nickel and cobalt in complex combination can likewise be used.

*Example 3.*—10 kgs. of knitted viscose are dyed at about 80° C. and for about 1 hour in 300 liter of a dyeing bath, containing 200 grams of the dyestuff which is obtainable by coupling diazotized 5-nitro-2-amino phenol and 2-naphthyl amine-5-sulfonic acid and boiling the thus obtained compound for several hours with at least an equimolecular quantity of chromium formate, said dyestuff having probably the following formula:



2 kgs. of Glauber's salt and 0.2 kg. of soap. Powerful even green shades of good fastness to light are obtained.

An even pink of good fastness properties is obtained by dyeing in the same manner as indicated above with a chromium compound of the dyestuff from diazotized 4-chloro-2-amino phenol-6-sulfonic acid and 1-(3'-sulfo-phenyl)-3'-methyl-5-pyrazolone; the chromium containing dyestuff from diazotized 1-amino-2-naphthol-sulfonic acid and 1-naphthol-8-sulfonic acid dyes an even clear blue shade; the dyestuff containing chromium obtainable from diazotized 2-amino-benzoic acid and 2-amino-naphthalene-7-sulfonic acid dyes an even violet tint; the zinc compound prepared from the dyestuff from diazotized 5-nitro-2-amino phenol and 2-(4'-methoxy-phenyl amino)-5-naphthol-7-sulfonic acid (coupled in the presence of alkali) dyes an even clear violet shade; the copper compound prepared from the dyestuff from diazotized 5-nitro-2-aminophenol and 2-(4'-ethoxy-phenyl-amino)-5-naphthol-7-sulfonic acid dyes an even deep reddish blue shade.

We claim:

1. The process which comprises dyeing viscose of different origin with an azodyestuff containing in ortho position to an azo group at least one substituent of the group consisting of hydroxy-, carboxylic acid-, alkoxy-, aralkoxy- and aldehydo groups or containing in its molecule at least one salicylic acid group, containing in complex combination a metal of the group consisting of copper, nickel, cobalt, chromium, cadmium, zinc, vanadium and iron.

2. The process which comprises dyeing viscose of different origin with an azodyestuff containing in ortho position to an azo group

at least one substituent of the group consisting of hydroxy-, carboxylic acid-, alkoxy-, aralkoxy- and aldehydo groups or containing in its molecule at least one salicylic acid group, containing chromium in complex combination.

3. The process which comprises dyeing viscose of different origin with a chromium complex compound of the azodyestuff prepared from diazotized 5-nitro-2-aminophenol and 2-naphthylamine-5-sulfonic acid.

4. As new articles of manufacture viscose of different origin dyed with an azodyestuff as claimed in claim 1; the dyeings being distinguished by an excellent evenness.

5. As new products of manufacture viscose of different origin dyed with an azodyestuff as claimed in claim 2, the dyeings being distinguished by an excellent evenness.

6. As a new article of manufacture viscose of different origin dyed with the azodyestuff as claimed in claim 3, the dyeing being distinguished by an excellent evenness.

25 In testimony whereof we have hereunto set our hands.

WINFRID HENTRICH. [L. S.]

MAX HARDTMANN. [L. S.]

JOSEF HILGER. [L. S.]

RUDOLF KNOCHE. [L. S.]

30

35

40

45

50

55

60

65